

April 23, 1940.

H. BRUINING ET AL

2,198,329

ELECTRIC DISCHARGE TUBE

Filed March 12, 1938

SECONDARY ELECTRON Emitter  
WITH LAYER OF ALKALINE EARTH  
METAL OXIDE NO THICKER THAN  
ONE MICRON AND SUBSTANTIALLY  
FREE OF METAL OF THE OXIDE



INVENTORS  
HAJO BRUINING AND  
JAN HENDRIK DE BOER  
BY

*Charles McClair*  
ATTORNEY.

## UNITED STATES PATENT OFFICE

2,198,329

## ELECTRIC DISCHARGE TUBE

Hajo Bruining and Jan Hendrik de Boer, Eindhoven, Netherlands, assignors, by mesne assignments, to Radio Corporation of America, New York, N. Y., a corporation of Delaware

Application March 12, 1938, Serial No. 195,567  
In the Netherlands March 25, 1937

3 Claims. (Cl. 250—174)

The invention relates to an electric discharge tube comprising a secondary-emission electrode, that is to say an electrode which is coated, at least on part of its surface, with a material which readily emits secondary electrons when it is struck by primary electrons.

In literature there are mentioned a large number of materials which possess this property. In most patents and publications reference is 10 made to metals and to compounds of alkali metals and alkaline earth metals, metallic caesium absorbed to caesium oxide being very customary.

Applicants have made extensive investigations on this subject and have found that, as 15 regards the value of the secondary emission, it is by no means indifferent whether use is made of compounds or of metals but that a very high secondary emission is only obtained if use is made of an electric discharge tube according to the 20 present invention which comprises a secondary-emission electrode coated, at least on part of its surface, with a layer which is not thicker than 1 micron and which consists of one or 25 more compounds of the alkali, alkaline earth or earth metals which do practically not contain 30 free metal. By alkali metals are meant the metals: lithium, sodium, potassium, rubidium and caesium, by alkaline earth metals the metals calcium, strontium, barium and in the present case also magnesium and by the earth metals: aluminium, scandium, yttrium, lanthanum and the rare earth metals, furthermore, zirconium, titanium, hafnium and thorium.

Applicants have found, in fact, that the generally accepted opinion that materials which have a satisfactory primary emission also will have the best secondary emission is incorrect but that the best secondary emission is only obtained if use is made of a layer which consists of one or more compounds in which there is practically no free metal, that is to say of a layer which would be completely unsuitable to act as a primary emitter. Based on this recognition the invention consists in the use of layers which consist of compounds which practically contain no free metal and which have a small thickness, which is necessary as the conductivity of such layers is smaller than that of layers which contain a more or less large amount of free metal.

50 Although different materials may be utilised for the purpose above referred to, use should preferably be made of oxides, or halogenides of the alkali metals, or alkaline earth metals such, for example, as barium oxide, caesium oxide, sodium chloride, potassium chloride, sodium fluoride, sodium bromide, potassium iodide, alumin-

ium oxide, etc. The table below indicates the values of the secondary emission for the above-mentioned compounds and for the pure metals.

| Material                       | Sec. emission | Voltage | 5  |
|--------------------------------|---------------|---------|----|
| BaO                            | 4.75          | 400     |    |
| Ba                             | 0.8           | 600     |    |
| Cs <sub>2</sub> O              | 4.2           | 200     |    |
| Cs                             | 0.72          | 400     |    |
| NaCl                           | 6.8           | 600     | 10 |
| NaBr                           | 5.6           | 300     |    |
| NaF                            | 5.7           | 300     |    |
| Na                             | 0.9           | 300     |    |
| KCl                            | 7.5           | 300     |    |
| KI                             | 5.4           | 300     |    |
| K                              | 0.9           | 300     |    |
| Al <sub>2</sub> O <sub>3</sub> | 3.0           | 300     | 15 |
| Al                             | 1.0           | 300     |    |

As may be seen from this table the secondary emission of the compounds is materially greater than that of the pure metal.

The accompanying drawing illustrates diagrammatically one embodiment of my invention as a tube comprising an envelope 1 enclosing a source of primary electrons, such as a thermionic cathode 2, a conventional control grid 3, an output electrode 4, and a secondary electron emitter 5 constructed in accordance with my invention and having a layer 6 of alkaline earth oxide on the surface facing the cathode. The primary electron stream flows, as indicated by a single arrow, from the source 2 to the emitter 5, and the secondary electron stream flows, as indicated by several arrows, from the emitter 5 to the output electrode 4.

What we claim is:

1. An electron discharge tube comprising a source of primary electrons, a collector electrode, and a secondary electron emitting electrode having on the surface exposed to said source a layer no thicker than one micron and consisting of an oxygen compound of a metal selected from the group consisting of the alkali and the alkaline earth metals and substantially free from the metal of the compound.

2. A secondary electron emitter for an electron discharge device comprising an electrode, and a coating on said electrode thinner than one micron and consisting of an oxide of an alkali or alkaline earth metal and free from the metal of the oxide.

3. A secondary electron emitter for an electron discharge device comprising an electrode, and a coating on said electrode no thicker than one micron and consisting of an oxide of an alkaline earth metal and free from said metal.

HAJO BRUINING.

JAN HENDRIK DE BOER.